

# UNITED STATES PATENT OFFICE.

EDWIN L. POWELL, OF NEW ORLEANS, LOUISIANA.

## WOOD-PRESERVING COMPOUND.

1,036,706.

Specification of Letters Patent. Patented Aug. 27, 1912.

No Drawing.

Application filed January 18, 1910. Serial No. 538,602.

*To all whom it may concern:*

Be it known that I, EDWIN L. POWELL, a citizen of the United States, residing at New Orleans, in the parish of Orleans and 5 State of Louisiana, have invented certain new and useful Improvements in Wood-Preserving Compounds; and I do declare the following to be a full, clear, and exact description of the invention, such as will enable others skilled in the art to which it 10 appertains to make and use the same.

The invention relates to compounds for preserving timber.

It has for its object to provide a compound 15 possessing preservative and antiseptic properties and which tends to solidify when injected into the pores of the wood, and which is insoluble in and practically unaffected by water, and practically unaffected 20 by atmospheric conditions as to heat, so far as concerns the larger percentage of the compound, thus producing a wood preservative compound having greater stability and possessing the necessary properties to 25 resist the disintegrating influences of bacteria and fungus life.

To the accomplishment of the objects stated the invention consists in the compound hereinafter described and particularly 30 specified in the claims.

The compound is formed by thoroughly mixing, under natural or artificial heat, preferably at a temperature of approximately 150° Fah., dead oil of coal tar, otherwise 35 known as creosote oil, and crude petroleum having an asphaltum base, in varying proportions. The proportion of creosote oil will largely be governed by the purposes for which the timber preserved with the mixture 40 or compound is to be used, a smaller proportion of creosote oil being employed where the compound is to be used in preserving timber used on land or in dry climates than where the timber is to be used 45 in wet climates, in swamps, in running water, or in salt water where protection is desired against the salt water worms and borers such as the *Teredo* and *Limnoria*. The proportions accordingly can be varied 50 within wide range. For cross ties and timbers used under ordinary conditions on land, the economical and effective mixture is 20% to 25% dead oil of coal tar (creosote) the balance being crude oil having an asphaltum 55 base. For piling and timbers used in water the mixture may be as high as 50% of each

constituent. The crude oil employed is preferably that which has had removed therefrom the ordinary kerosene oil and if desired also lubricating oil and gasoline by 60 distillation under any of the well known methods in use, or there may be employed crude petroleum having an asphaltum base from which kerosene, gasoline and lubricating oils have been removed by the ordinary 65 well known methods in use for that purpose. In all cases however an essential ingredient of the compound is crude petroleum having an asphaltum base, mixed with dead oil of coal tar, or creosote oil. 70

Creosote oil or dead oil of coal tar, is the best known wood preservative, and is both antiseptic and waterproofing in its action. Crude oil having an asphaltum base is also 75 antiseptic and the heavy portions thereof fill the wood cells and prevent the entrance of water.

The compound described has been found to contain approximately 90% of a stable body which coagulates or solidifies in the 80 wood cells, practically filling the cells and to a material degree remaining unaffected by atmospheric conditions or heat, and insoluble in and practically unimpaired or unaffected by water, thus affording a waterproof 85 as well as a preservative compound for timber, which materially prolongs the life of the timber, and at the same time possessing the beneficial result derived from the use of creosote or dead oil of coal tar, 90 and at a materially smaller cost. The reduction in cost is very important, as the amount of treated timber used is almost wholly governed by the cost of treatment.

The compound may be applied to the timber by methods well known in the preservation of wood by injecting preservatives into the wood cells. 95

Having described my invention and set forth its merits, what I claim is:— 100

1. A wood-preserving compound containing dead oil of coal tar, or creosote oil, and a material containing at least the higher boiling constituents of crude petroleum having an asphaltum base. 105

2. A wood-preserving compound containing dead oil of coal tar, or creosote oil, and crude petroleum having an asphaltum base from which kerosene oil and gasoline have been removed. 110

3. A wood-preserving compound containing dead oil of coal tar, or creosote oil, and

crude petroleum having an asphaltum base from which kerosene, gasolene, and lubricating oils have been removed.

4. A wood preserving compound containing creosote oil and a material containing the still bottoms of asphaltic petroleum.

5. A wood preserving compound consisting of 1 part of creosote oil and from 1 to 3 parts of a material containing the still bottoms of asphaltic petroleum.

6. A wood preserving compound contain-

ing 1 part of creosote oil and 1 to 3 parts of asphaltic petroleum from which the kerosene, gasolene and lubricating oils have been removed.

In testimony whereof I affix my signature in presence of two witnesses.

EDWIN L. POWELL.

Witnesses:

JAS. SIMEON,  
EDWARD WATERMEIER.